

March 24, 1959

P. W. NIPPERT ET AL  
METHOD OF PRODUCING HEAT TREATED COPPER ZIRCONIUM  
ALLOYS AND ARTICLES FORMED THEREOF  
Filed June 23, 1958

2,879,191



Fig. 1.



Fig. 2.



Fig. 3.

Fig. 4.

INVENTOR.  
PAUL W. NIPPERT  
BY  
Schmieding and Fultz  
ATTORNEYS

METHOD OF PRODUCING HEAT TREATED  
COPPER ZIRCONIUM ALLOYS AND ARTI-  
CLES FORMED THEREOF

Paul W. Nippert, Worthington, and Allen W. Hodge, Columbus, Ohio, assignors to The Nippert Electric Products Company, Columbus, Ohio, a corporation of Ohio

Application June 23, 1958, Serial No. 744,313

8 Claims. (Cl. 148—11.5)

This invention relates to copper-zirconium alloys, and methods for producing same, and particularly to a novel copper-zirconium alloy for the production of improved electrical conductors such as commutators and the like.

This application is a continuation-in-part of our pending application Serial No. 674,086, filed July 25, 1957, now abandoned, which is a continuation-in-part of Serial No. 603,984, filed August 14, 1956, now abandoned.

In general, the method of the present invention provides an improved copper-zirconium alloy that not only retains excellent strength and electrical conductivity characteristics, at elevated temperatures, but also possesses the unique characteristic, for copper base alloys, of being stronger in a transverse-to-cold-working direction than in a parallel-to-cold-working direction.

Silver-bearing copper alloys and chromium-copper alloys have been found to possess good electrical characteristics when used to fabricate electrical conductors for use at elevated temperatures but such alloys, when subjected to cold working, are not strengthened in a transverse-to-cold-working direction, as compared to a parallel-to-cold-working direction, and hence do not possess the above mentioned unique physical characteristic of the novel copper-zirconium alloy of the present invention. Moreover, copper-zirconium alloys, produced prior to the novel method of the present invention, are like the above mentioned silver-bearing copper and chromium-copper alloys in that such copper-zirconium alloys do not become stronger in a transverse-to-cold-working direction than in a parallel-to-cold-working direction.

In addition to the above, the novel copper-zirconium alloy of the present invention possesses another unusual physical characteristic in that it is not notch sensitive. That is, a notched electrical conductor, such as a commutator segment, formed from the copper-zirconium alloy of the present invention, is not weakened by the presence of the notches. In contrast, notched electrical conductor formed of silver-bearing copper or chromium-copper alloys possess great notch sensitivity in that the conductor is very materially weakened by the presence of the notches.

It is therefore an object of the present invention to provide a novel copper-zirconium alloy, and method for producing same, which alloy is stronger in a transverse-to-cold-working direction as compared to a parallel-to-cold-working direction.

It is another object of the present invention to provide a novel copper-zirconium alloy, and method for producing same which alloy can be used to form notched articles that are not weakened by the presence of the notches.

It is another object of the present invention to provide a novel copper-zirconium alloy having high strength and high electrical conductivity at elevated temperatures, and a novel method for producing said alloy whereby the grain growth and hence grain size of the alloy can be

selectively varied without materially reducing said high strength and high electrical conductivity.

It is another object of the present invention to provide an improved electrical conductor, for use at elevated temperatures, which conductor is formed by cold working and is stronger in the transverse-to-cold-working direction than in the parallel-to-cold-working direction.

It is still another object of the present invention to provide an improved electrical conductor, for use at elevated temperatures, which conductor is provided with notches but not weakened by the presence thereof.

Further objects and advantages of the present invention will be apparent from the following description, reference being had to the accompanying drawings wherein a preferred form of embodiment of the invention is clearly shown.

In the drawing:

Figure 1 is a perspective view of a typical commutator formed of segments each of which segments constitutes an electrical conductor fabricated according to the present invention;

Figure 2 is a perspective view of a rolled plate formed from the novel copper-zirconium alloy of the present invention and according to the novel method thereof. Transversely disposed specimens for demonstrating the advantages of the present invention are cut from the rolled plate in the manner designated by dotted delineation thereon;

Figure 3 is a perspective view of a first type of test specimen formed from the novel copper-zirconium alloy of the present invention, said specimen having been cut from a plate of the type illustrated in Figure 2; and

Figure 4 is a perspective view of a second type of test specimen formed from the novel copper-zirconium alloy of the present invention, said specimen having been cut from a plate of the type illustrated in Figure 2.

Reference is next made to Figure 1 of the drawings which illustrates a typical commutator installation. For many years the development of small, high-speed motors, employing commutators of the same general type as Figure 1, was limited by the low strength of substantially pure, hard-rolled copper commutators. Investigations showed that the strength of tough-pitch copper at high temperatures could be increased considerably without loss of electric conductivity by small additions of silver. The addition of 25 to 35 oz. of silver per ton of coarse-grained, hard-rolled copper extended the strength of commutators to prolonged exposures at 390° F. and short-time exposures as high as 750° F.

Up to World War II, this alloy was able to withstand higher temperatures than the best available insulating materials. When better insulating materials were developed, however, commutator design was again held back by the softening of copper at elevated temperatures. Experience indicates that 450° F. is the highest operating temperature permissible for motors equipped with silver-copper commutators.

Chromium-copper then was investigated and found suitable for commutators operating at or above 500° F. (260° C.). Use of this alloy also presented a number of problems. Chromium-copper is extremely difficult to cast into good, solid wire bar, and die wear in drawing is extremely severe due to the undissolved chromium and oxide stringers.

Also, if used in the fully heat-treated condition, chromium-copper commutator segments have a tendency to crack at the dovetails. Typical commutator segments 20 provided with dovetails 22 are illustrated in Figure 1. To prevent cracking of segments formed of chromium-copper, it is necessary to heat-treat the bars and lower their hardness below the brittle stage. This operation is very critical since it is necessary to exceed the minimum recrys-

tallization temperature for a period of time that must be determined individually for each batch of copper and each bar size. It is also necessary to check the bar hardness before and after heat treatment. The loss of chromium-copper from both over-softening and from poor original casting runs from 10 percent to as high as 80 percent of the total metal processed.

Commutator segments are subject to stresses from the forces exerted by the clamping or V-ring 24, Figure 1, and from the centrifugal forces generated by high speed rotation. Increasing temperatures decrease the ability of the segments to withstand these stresses. In extreme cases, the increased temperature causes the metal to deform and the segments to be thrown out. Even segment movement of a few ten-thousandths of an inch will cause excessive brush wear. If the metal remains hard, but loses strength and ductility, the segments may crack. Failure of any segment, either by excessive deformation or by cracking, will cause complete motor failure.

During motor rotation, the stresses set up by centrifugal force are transverse to the direction in which the commutator segment 20 is rolled, such direction of cold working being diagrammatically represented by an arrow 25 in Figure 1. Such stresses are also across the dovetail 22 that constitutes part of the commutator design. These centrifugal forces may be augmented by slight distortions resulting from the heavy compression forces exerted on the ends of the segments 20 by the locking rings 24. Since the thermal expansion of copper is greater than that of steel, the assembly compression forces become greater when the temperature rises. In general, cracks in segments of chromium-copper commutators invariably appear to have been tensile failures in the transverse-to-rolling direction.

The novel copper-zirconium alloy of the present invention does not possess the above mentioned disadvantages and hence is highly desirable for the fabrication of superior electrical conductors for use at relatively high temperatures.

It has been discovered that the superior alloy of the present invention can be produced as follows:

A percentage of from .01 to .15 zirconium and the balance electrolytically refined copper are alloyed in a suitable manner.

Electrolytically refined copper suitable for practicing the present invention, as employed in the claims herein, is defined in ASTM Standards for Electrolytic Copper, 1955 edition, part 2, paragraph B-224-52 as copper having 100 percent conductivity at 20 degrees centigrade and again at paragraph B5-43 as 99.900 copper and silver (silver being counted as copper) having a resistivity of .15328 international ohm per meter-gram at 20 degrees centigrade.

It will be understood that refined copper that is refined by means other than electrolytic means can be used in practicing the present invention provided such refined copper has an electrical conductivity equal to the electrical conductivity of electrolytically refined copper.

The resulting alloy is next solution annealed at a temperature between 1300 degrees and 1900 degrees Fahrenheit for from five to sixty minutes. The solution annealed alloy is then quenched to produce a rapid reduction in temperature after which it is cold worked, preferably to the extent that a fifty percent reduction in cross-sectional area is produced by such cold working.

A preferred composition for practicing the method of the present invention consists of an alloy of substantially .08 zirconium and the balance copper.

At solution annealing temperatures below 1300 degrees Fahrenheit the strength developed subsequently by the copper-zirconium alloy is too low for efficient utilization of the potential of the invention. At substantially 1400 degrees Fahrenheit the optimum increase in strength in the transverse-to-cold working direction is realized.

As still another unusual and useful characteristic, the

alloy of the present invention can be solution annealed at various temperatures, throughout the previously mentioned range of 1300 degrees to 1900 degrees Fahrenheit, so as to selectively control grain growth to produce the desired grain size in the finished work. In solution annealing the alloy of the present invention at the various temperatures it has been found that the high strength and high electrical conductivity of the present alloy are not materially affected. Since grain growth is a function of time, as well as temperature, the time at temperature can also be varied throughout a corresponding broad range to control grain growth without materially affecting the above mentioned characteristics. To the knowledge of the present inventors no other copper base alloy can be solution annealed at various temperatures throughout a range but must be treated at certain time-temperature relationship in order to obtain the desired strength and electrical conductivity characteristics. Hence the flexibility in controlling grain size is not present. It will therefore be understood that the above described solution annealing range of the alloy of the present invention is particularly useful where large batches of the alloy are to be uniformly heated throughout thus enabling the central portions of the batches to be gradually brought up to a selected low solution annealing temperature, say 1300 degrees-1500 degrees Fahrenheit, without excessive heating and hence excessive grain growth occurring in the surface portions of the batches.

It has further been discovered that the electrical conductivity of the novel copper-zirconium alloy of the present invention can be increased to the high value of about ninety-five percent of the electrical conductivity of pure copper. This increase in electrical conductivity may be effected by aging the alloy in a furnace either after the previous mentioned solution anneal and quench steps, or after the previously mentioned cold-working step. Maximum increases in electrical conductivity are realized when the alloy is aged at between 450 degrees and 950 degrees Fahrenheit and preferably for a period of between 60 and 120 minutes.

To evaluate the strength of the present alloy, both tensile and creep-rupture tests were performed. In the tensile test, the metal was loaded at a comparatively rapid rate to failure. In the creep-rupture test, delayed failure is brought about at lower load levels.

Because some metals exhibit great sensitivity to notches, accidental scratches or a designed notch such as thread on a bolt, both notched specimens 27 and unnotched specimens 28 were used for each test, see Figures 3 and 4. Specimens for each test were taken from both the parallel-to-rolling and transverse-to-rolling directions. Such transversely disposed specimens are indicated at 28-A and 28-B, respectively, in Figure 2, with such specimens being cut from a rolled plate 31. The direction of rolling or cold working of plate 31 is diagrammatically indicated by an arrow 25.

Notched bars were used in the rupture tests to indicate the properties of the metal that could be expected in a commutator.

Some mechanical properties of the present novel alloy, both at room temperature and at 550° F. (299° C.), are shown in Table I set forth at the end of the present specification. These properties were determined after the alloy had been given the proper amount of cold work and heat-treatment to produce the hardness noted. For comparison, the properties at 550° F. of silver-bearing copper and of chromium-copper at the usual hardness levels are shown in Table II. The electrical conductivity of the three commutator alloys is shown in Table III.

The softening temperatures of both cold-worked and aged alloy of the present invention and of commercial chromium-copper, after exposures of 1/2 hour is about 930° F. (500° C.). Silver-bearing copper (25 oz. per ton) softens from 600 to 625° F. (315 to 330° C.). In service, commutator segments are usually exposed to

lower temperatures; cumulative exposure times, however, may be much longer.

Rupture tests were made to determine the strength of the commutator alloys under extended loading times at elevated temperatures, Table IV. As indicated, the rupture strength of all of the alloys decreased at the elevated temperature. Silver-bearing copper exposed to 550° F. (288° C.) for 100 hr. or more was permanently damaged and lost much of its strength. Chromium-copper evidenced great notch sensitivity, although it retained considerable strength in the parallel-to-rolling direction. In the transverse-to-rolling direction, the rupture strength was approximately that of softened silver-bearing copper. Chromium-copper did not soften permanently.

Quite different results were obtained with the zirconium-copper alloy of the present invention. First, the notches strengthened the copper-zirconium alloy bars that were loaded in either direction, transverse or longitudinal. Second, specimens loaded in the transverse-to-rolling direction were stronger than corresponding specimens loaded in the parallel-to-rolling direction. Unnotched bars, after 500 hr. of sustained loading in the longitudinal direction at 550° F. retained 76 percent of their original tensile strength. Under each of the conditions of loading, they were still stronger.

It can be noted also that the time-rate of loss of strength of alloy of the present invention was very much less than the other two alloys.

Another property of primary importance is the ability of a commutator alloy to develop and maintain a commutation film. Commutation tests show that brush life (both at sea level and at high altitudes) on commutators, fabricated from the alloy of the present invention, is at least equal to the brush life on similar commutators of silver-bearing copper or chromium-copper.

TABLE I

Typical mechanical properties of the zirconium-copper alloy produced according to the present invention

|                                                     | 75° F.     | 550° F. |
|-----------------------------------------------------|------------|---------|
| Specimens taken in parallel-to-rolling direction:   |            |         |
| Hardness, Rockwell B.....                           | 46         |         |
| Tensile strength, p.s.i.....                        | 53,500     | 42,000  |
| Yield strength, 0.2% offset, p.s.i.....             | 50,500     | 40,000  |
| Proportional limit, p.s.i.....                      | 19,000     |         |
| Modulus of elasticity, p.s.i.....                   | 18,700,000 |         |
| Elongation, percent in 2 in.....                    | 10.6       | 7.5     |
| Reduction in area, percent.....                     | 54.3       |         |
| Specimens taken in transverse-to-rolling direction: |            |         |
| Hardness Rockwell B.....                            | 66         |         |
| Tensile strength, p.s.i.....                        |            | 44,000  |
| Yield strength, 0.2% offset, p.s.i.....             |            | 41,500  |
| Elongation, percent in 2 in.....                    |            | 6.5     |

TABLE II

Typical mechanical properties of silver-bearing copper and chromium-copper at 550° F. (288° C.)

|                                           | Silver-bearing Copper | Chromium Copper |
|-------------------------------------------|-----------------------|-----------------|
| Hardness, Rockwell B (at room temp.)..... |                       |                 |
| Parallel-to-rolling direction:            |                       |                 |
| Yield strength, 0.2% offset, p.s.i.....   | 28,000                | 46,000          |
| Tensile strength, p.s.i.....              | 35,000                | 50,000          |
| Reduction of area, percent.....           | 42.5                  | 4               |
| Elongation, percent in 2 in.....          | 12                    | 7               |
| Transverse-to-rolling direction:          |                       |                 |
| Yield strength, 0.2% offset, p.s.i.....   | 31,000                | 41,000          |
| Tensile strength, p.s.i.....              | 36,000                | 47,000          |
| Reduction in area, percent.....           | 25.5                  | 6               |
| Elongation, percent in 2 in.....          | 8                     | 3               |

TABLE III  
Electrical conductivity of copper alloys at 68° F. (20° C.)

|                                                | Percent |
|------------------------------------------------|---------|
| 5 International annealed copper standard ..... | 100.0   |
| Silver-bearing copper, Rockwell 61 B .....     | 97.0    |
| Zirconium-copper alloy of the invention:       |         |
| Rockwell 68 B .....                            | 95.8    |
| Chromium-copper, Rockwell 82 B .....           | 82.0    |

TABLE IV

Typical rupture strengths of commutator alloys at 550° F. (288° C.)

| 15                                           | After 100 hr., p.s.i. |         | After 500 hr., p.s.i. <sup>1</sup> |         |
|----------------------------------------------|-----------------------|---------|------------------------------------|---------|
|                                              | Un-notched            | Notched | Un-notched                         | Notched |
| 20 Parallel-to-rolling direction:            |                       |         |                                    |         |
| Zirconium-copper alloy of the Invention..... | 34,000                | 37,500  | 32,000                             | 35,500  |
| Chromium-copper.....                         | 36,000                | 28,000  | 32,500                             | 23,500  |
| Silver-bearing copper.....                   | 17,500                | 15,500  | 10,500                             | (2)     |
| 25 Transverse-to-rolling direction:          |                       |         |                                    |         |
| Zirconium-copper alloy of the invention..... | 38,000                | 41,500  | 36,500                             | 38,500  |
| Chromium-copper.....                         | 18,500                | 17,000  | 13,000                             | 12,000  |
| Silver-bearing copper.....                   | 20,000                | 15,500  | 14,000                             | (3)     |

<sup>1</sup> Values extrapolated to 500 hr. from tests running up to 350 hr.

<sup>2</sup> Rupture strength approximately 10,000 p.s.i. after 210 hr., and decreasing rapidly.

<sup>3</sup> Rupture strength approximately 10,000 p.s.i. after 300 hr., and decreasing rapidly. Rupture strength of silver-bearing copper, unnotched, after 500 hr. is estimated only. Recrystallization and softening of the metal, very noticeable in the notched specimens, might make these apparent values higher than the true values.

EXPERIMENTS TO DETERMINE THE RELATIONSHIP  
35 BETWEEN HARDNESS AND AGING TIME OF SUPER-SATURATED COPPER-ZIRCONIUM ALLOYS

Reference is made to U.S. Patent No. 2,097,816 issued to Hensel et al. on November 2, 1937.

The Hensel patent shows by a curve (line 10, Figure 40) how an alloy described as copper-1 percent zirconium that has been quenched from 950° centigrade (1742 degrees Fahrenheit) increases in hardness on artificial aging at 450° centigrade (842 degrees Fahrenheit). Points read from the curve show approximately the following values:

|                                         | Aging Time, hours | Hardness, Rockwell B |
|-----------------------------------------|-------------------|----------------------|
| 50 As quenched.....                     | 0                 | 0                    |
| 0 (presumably after natural aging)..... | 10                | 10                   |
| 1.....                                  | 42                | 42                   |
| 2.....                                  | 53                | 53                   |
| 4.....                                  | 58                | 58                   |
| 8.....                                  | 58                | 58                   |
| 16.....                                 | 53                | 53                   |

55 Two alloys were prepared in accordance with the present invention, using electrolytically refined copper and a copper-zirconium master alloy that was prepared from commercial (Kroll process) zirconium sponge available in 1957. These two zirconium-copper alloys were rolled to bar, annealed at 950° centigrade (1742 degrees Fahrenheit) and aged at 450° centigrade (842 degrees Fahrenheit). One of these alloys contained 0.22 percent of zirconium, the other 1.0 percent.

65 The average hardness values obtained from these two alloys were approximately alike, as shown below. This was expected because the amount of zirconium present in each case exceeded the limit of solubility of zirconium in copper. This limit is now believed to be about 0.15 percent at 1896 degrees Fahrenheit (980° C.).

70 When zirconium is referred to hereinafter in connection with the alloy of the present invention, the term "zirconium" means zirconium at least equal in purity to the commercial Kroll process zirconium mentioned above.

| Aging Time, hours | Hardness, Rockwell B |               |
|-------------------|----------------------|---------------|
|                   | 0.22% Zr Alloy       | 1.0% Zr Alloy |
| 0                 | 16.1                 | 20            |
| 1                 | 24.7                 | 22            |
| 2                 | 26.8                 | 25            |
| 4                 | 26.3                 | 27            |
| 8                 | 28.8                 | 27            |
| 16                | 28.0                 | 31            |

When plotted, both sets of data indicate a maximum hardness of about Rockwell B 30. Since the determinations were made at different times, the differences are more probably caused by small errors in the Rockwell B readings than by differences in the hardness of the alloys. (The Rockwell B scale is not well adapted to making hardness determinations on so soft a metal.)

There is almost no relationship between the aging response of these two zirconium alloys made in 1957, which have a maximum hardness of about Rockwell B 30, and the alloy described in U.S. Patent 2,097,816, which had a maximum hardness of about Rockwell B 58. The alloy described in the patent cited showed a vigorous response to age hardening, while the two alloys produced according to the present invention show a relatively feeble response. That these striking differences, which suggest entirely different alloys, are not caused by small differences in the zirconium content is demonstrated by the similar response of the two alloys of widely different composition made in 1957.

Only a conjecture as to the cause of the hardening behavior of the alloy described in U.S. Patent 2,097,816 can be advanced. Zirconium available at the time the patent was issued (1937) probably was produced by aluminothermic reduction and may have contained important quantities of silicon, titanium, iron, aluminum, and possibly other impurities such as nickel or chromium. Quite possibly the iron, nickel, etc., may have combined with the silicon, the titanium, or even with a part of the zirconium, to form compounds which could be precipitated from solution during aging. This fortuitous hardening produced an alloy suitable for making welding electrodes. On the other hand, the impurities increased the electrical resistance of the unaged alloy to less than 50 percent I.A.C.S. Line 11 of Figure 1 of the patent shows that the conductivity could be increased by aging at 450° centigrade (842 degrees Fahrenheit) to about 73 percent I.A.C.S. at the maximum hardness, and to a maximum of about 78 percent I.A.C.S. by severely over aging (32 hours or more at 450° centigrade (842 degrees Fahrenheit).

Ultra-high quality commutators demand an alloy with good thermal stability and with an electrical conductivity of 90 percent I.A.C.S. or higher. The teachings of U.S. Patent 2,097,816 do not suggest that such an alloy could be produced from zirconium-copper. Rather, they tend to show that a very high conductivity alloy could not be produced from an alloy of copper with zirconium. Since high-conductivity (more than 90 percent I.A.C.S.), thermally stable alloys have been produced from binary alloys of copper and zirconium, and since these alloys do not show the response to artificial aging of the alloy described in the patent cited, it is believed that the alloy described in the patent was not a binary alloy of copper and zirconium, but that it contained other elements fortuitously introduced as impurities. Moreover, it is believed that these impurities were largely responsible for the behavior of the alloy during artificial aging and for its mechanical and electrical properties.

While the form of embodiment of the present invention as herein disclosed constitutes a preferred form, it is to be understood that other forms might be adopted, all coming within the scope of the claims which follow.

We claim:

1. The steps in the method of producing an improved metal alloy for cold working which alloy possesses greater strength in a direction transverse to the direction of cold working, said method comprising alloying about .01 to about 1.0 percent zirconium and the balance electrolytically refined copper; solution annealing said alloy at a temperature between 1300 degrees and 1740 degrees Fahrenheit; quenching said alloy; and subjecting said alloy to cold working.

2. The steps in the method of producing an improved metal alloy for cold working which alloy possesses greater strength in a direction transverse to the direction of cold working, said method comprising alloying about .01 to about 1.0 percent zirconium and the balance refined copper having an electrical conductivity equal to that of electrolytically refined copper; solution annealing said alloy at a temperature between 1300 degrees and 1740 degrees Fahrenheit; quenching said alloy; and subjecting said alloy to cold working.

3. The steps in the method of producing an improved metal alloy for cold working which alloy possesses greater strength in a direction transverse to the direction of cold working, said method comprising alloying about .01 to about .15 percent zirconium and the balance refined copper having an electrical conductivity equal to that of electrolytically refined copper; solution annealing said alloy at a temperature of substantially 1400 degrees Fahrenheit; quenching said alloy; and subjecting said alloy to cold working.

4. The steps in the method of producing an improved metal alloy for cold working which alloy possesses greater strength in a direction transverse to the direction of cold working, said method comprising alloying about .08 percent zirconium with the balance refined copper having an electrical conductivity equal to that of electrolytically refined copper; solution annealing said alloy at a temperature between 1300 degree and 1740 degrees Fahrenheit; quenching said alloy; and subjecting said alloy to cold working.

5. The steps in the method of producing an improved metal alloy for cold working which alloy possesses greater strength in a direction transverse to the direction of cold working, said method comprising alloying about .01 to about .15 percent zirconium and the balance refined copper having an electrical conductivity equal to that of electrolytically refined copper; solution annealing said alloy at a temperature between 1300 degrees and 1740 degrees Fahrenheit; quenching said alloy; and subjecting said alloy to cold working.

6. An electrical conductor made of a cold worked alloy of about .01 to about 1.0 percent zirconium and the balance refined copper having an electrical conductivity equal to that of electrolytically refined copper, said alloy having an electrical conductivity in excess of 90 percent.

7. An electrical conductor having an electrical conductivity greater than 80 percent I.A.C.S. made of a cold worked alloy of about .01 to about .15 percent zirconium and the balance refined copper having an electrical conductivity equal to that of electrolytically refined copper.

8. An electrical conductor made of a cold worked alloy of about .08 percent zirconium and the balance electrolytically refined copper, said alloy having an electrical conductivity in excess of 90 percent.

#### References Cited in the file of this patent

#### UNITED STATES PATENTS

- 2,097,816 Hensel et al. \_\_\_\_\_ Nov. 2, 1937  
 2,842,438 Saarivirta et al. \_\_\_\_\_ July 8, 1958  
 2,847,303 Pruna \_\_\_\_\_ Aug. 12, 1958

#### OTHER REFERENCES

- Metals Handbook, 1948 edition by American Society for Metals, page 858.